

June 24, 1930.

H. C. HARRISON

1,768,358

ELECTROLYTIC PROCESS AND APPARATUS

Filed May 21, 1925

2 Sheets-Sheet 1



INVENTOR

Herbert C. Harrison,  
Spencer, Dewitt, Hardman,  
ATTORNEYS.

June 24, 1930.

H. C. HARRISON

1,768,358

## ELECTROLYTIC PROCESS AND APPARATUS

Filed May 21, 1925

2 Sheets-Sheet 2



Fig. 8.



Fig. 6.



Fig. 7.

INVENTOR  
BY *Herbert C. Harrison*  
*Spencer, Pewsey & Harrison*  
ATTORNEYS

## UNITED STATES PATENT OFFICE

HERBERT CHAMPION HARRISON, OF LOCKPORT, NEW YORK; FLORENCE M. HARRISON, ARTHUR B. B. HARRISON, AND WILLIAM W. CAMPBELL, EXECUTORS OF SAID HERBERT CHAMPION HARRISON, DECEASED

## ELECTROLYTIC PROCESS AND APPARATUS

Application filed May 21, 1925. Serial No. 31,922.

This invention relates to a process and apparatus for electrolytically depositing metals, such as copper, of good physical quality, at a rate of speed hitherto deemed 5 impracticable commercially.

It has been well recognized for at least twenty-five years, that in order to obtain a coherent deposit of copper or other metal of good quality upon a cathode surface in an 10 electrolytic cell, it is necessary to maintain the concentration of the layer of electrolyte immediately in contact with the cathode, so that impoverishment of the electrolyte does not occur, since a given current of electricity 15 flowing for a given time always deposits the same amount of a given element from an electrolyte, providing the layer of electrolyte next to the cathode is not impoverished. For the purpose of obtaining rapid deposition 20 upon the cathode it is, therefore, necessary to utilize high current densities and to renew the concentration of the electrolyte with a rapidity to accord with the current density. Unless concentration of the electrolyte is maintained, high current densities 25 are ineffective to deposit pure coherent metal on the cathode.

The history of the art of electro-deposition shows that relatively high-rate copper 30 deposition has been possible for many years, although accompanied by physical limitations that have impeded commercial production while not inhibiting it altogether.

In the prior art, in so far as I am aware, 35 the cathode and anode containing portions of the cell have been so related that the electrolyte can pass freely from one portion to the other, both portions open to the atmosphere and both under atmospheric pressure. In 40 cells of this character both cathode and anode compartments being open to atmosphere, it is not practicable to effect rates of circulation required to utilize successfully current densities much in excess of 200 am- 45 peres per square foot.

I believe that I have solved the problem 50 of utilizing extremely high current densities, by injecting into the art a new principle. In the process of this application, the cathode is 55 completely separated from the anode or

anodes by, and is enclosed in, a tunnel-like chamber open only at opposite ends for the admission and escape of electrolyte and for the passage of the cathode, which may be a moving ribbon of indefinite length. The wall 55 of this cathode-enclosing chamber is of porous, non-conducting material, permeable to the electric current when saturated with electrolyte, which acts as the conducting medium between the anode and the cathode. 60 The chamber serves as an efficient guide to direct a stream of electrolyte in contact with the entire surface of the cathode, while at the same time serving to allow a small pre- 65 determined proportion of the electrolyte, say ten per cent, to pass through and form a second stream of lower velocity, flowing through the anode compartment or compartments. This tunnel-like cathode compartment should conform in cross section to the 70 cross section of the cathode inclosed by it. When a ribbon-like cathode is used, as contemplated, the compartment in cross section would have the form of a narrow slot, hav- 75 ing not more than one-sixteenth inch clearance on each side of the ribbon cathode. The electrolyte liquor is intended to be forced under pressure by a pump or head of electrolyte through this restricted cathode pas- 80 sage. Heads of from three feet to thirty feet may be used, whereby a speed through the cathode compartment of from ten to forty feet a second can be obtained, the pres- 85 sure dropping on the passage of the electrolyte through the compartment only slightly when once the speed of the stream is at- 90 tained. At the same time, the porosity of the inclosing wall acts as a pressure reducing valve, allowing the small proportion of 95 the electrolyte required to percolate through it into the anode compartment or compartments, which is or are at atmospheric or at least lower pressure than the cathode cham- 100 ber and in which the rate of flow is much reduced.

It is possible by this mode of procedure to effect satisfactory deposition of copper, for example, at rates as high as 2,000 am- 100 peres to the square foot, although it is ob- 105 vious that with such high rates the voltage

required to effect deposition will be increased, according to the condition of the cell.

In the accompanying drawings, in which like references indicate like parts throughout the several views, there is illustrated for the purpose of exemplification merely, apparatus by which the process may be practiced. In said drawings

10 Fig. 1 is a side view, partly in vertical section, illustrating an apparatus adapted to practice the process described;

15 Fig. 2 is a cross section of the electrolytic cell forming a part of the apparatus, taken on the line 2—2 of Fig. 1;

Fig. 3 is a cross section on the line 3—3 of Fig. 1;

15 Fig. 4 is a cross section on the line 4—4 of Fig. 1;

20 Fig. 5 is a plan view, partly in section, of the apparatus, but without the elevated tank for affording a pressure head for the electrolyte; the pump delivery pipe to said reservoir, and the stand pipe leading therefrom being shown in section.

25 Fig. 6 is a section on the line 6—6 of Fig. 5, looking to the left;

30 Fig. 7 is a cross section of a fragment of the tunnel-like cathode compartment of about full width; and

Fig. 8 is a longitudinal section through a fragment of the cathode compartment.

35 The apparatus here exemplified in Figs. 1 and 5 as one that is suitable to practice the process disclosed consists of the following main elements, namely: An electrolytic cell proper, 10, with certain directly connected appurtenances; a drip pan or catch tank 11 to receive the electrolyte discharged

40 from the cell; an elevated reservoir 12 to hold a head of electrolyte; a pump 13 with intake pipe 14 leading from the catch pan 11 and discharge pipe 15 delivering to the elevated reservoir 12; a stand-pipe 16 adapted to deliver the electrolyte from the reservoir 12 into and through the cell with high velocity; a delivery spool or reel 17 for receiving a roll of ribbon-like cathode of indefinite length, and a power-driven reel 18,

45 to wind up the compound strip comprising the cathode ribbon and adhering layers of deposited metal, and draw the cathode strip at any predetermined rate of speed through the cell.

50 The cell 10, as well as other parts that come in contact with the electrolyte, may be constructed of any suitable acid-proof material known for the purpose. The walls of the cell may be made, for example, of wood, lined with lead, of soapstone, acid-proof brick or tile, glass or vulcanite; and certain attachments, subject to contact with the electrolyte, may be made of any of the materials mentioned or any other suitable substance. The cell proper, 10, is confined

within the side walls 19, front end wall 20, rear end wall 21, and bottom 22, of an elongated box. The front end wall 20 and the rear end wall 21 are slotted vertically. The slot in the rear wall 21 is indicated at 70 23 in Fig. 3. Both slots are preferably of identical size and form and they are in alignment, preferably in the vertical mid plane of the cell. The slots 23 are for the purposes of receiving the cathode ribbon 24, 75 permitting its passage through the cell, and allowing the electrolyte 25 to enter and leave the cell. In dimensions the slots conform closely to the cross sectional dimensions of the cathode ribbon 24, being but very slightly longer than the width of the ribbon and of a width to allow not more than about one-sixteenth of an inch space on each side of the ribbon. The ribbon may be of standard rolled stock, eight inches in width, five one-thousandths of an inch in thickness, and of indefinite length. These dimensions have been found suitable for my purposes, but any practicable dimension of cathode ribbon may be used.

Extending longitudinally of the cell in alignment with the slots 23 is a cathode compartment of tunnel-like form 27, completely separated from the anode compartment, which occupies the remainder of the space 90 within the cell. This tunnel-like cathode compartment is formed as a flat tube, oblong in cross section, the ends of which are seated snugly in grooves 58 in the end walls 20 and 21. The passage or chamber 26 100 within the tunnel compartment is substantially of the same dimensions in cross section as slots 23. Within the passage 26 of compartment 27 there are, preferably, centering guides 28, having V-shaped notches to 105 guide and assist in centering the cathode ribbon within the compartment. These guides may be made of agate or other hard, acid-proof substance. In order to avoid, by any peculiar mischance, contact between the 110 sides of the ribbon cathode and the walls of the tunnel, other agate or like guides 28<sup>a</sup> of button-form may be imbedded partially in said walls. There may be three or more guides 28 at the bottom of the passage and an equal number at the top. The walls of the cathode tunnel should consist of a material that is porous enough to permit the slow passage of electrolyte through it, and I refer to it herein as a material that is semi-permeable to the electrolyte. It should be a poor conductor of electricity, but easily permeable to the electric current when saturated with electrolyte. One substance that fulfills these conditions is corborundum comminuted and having the granules bound together by a suitable cement, such as bakelite. In so far as its functional efficiency is concerned, the cathode compartment may be molded in one integral mass, or built up of 115 120 125 130

slabs. For convenience of manufacture I have constructed it of assembled slabs, cemented at the joints. It has already been said that the cathode tunnel conforms approximately in cross section to the cathode ribbon, being but slightly wider than the thickness of said ribbon. Three feet is a suitable length, but this dimension may be varied, like the others, as dictated by the necessities of use.

The anode compartment occupies the space on both sides of the cathode compartment, and the electrolyte, when the apparatus is in operation, stands above the top of the cathode compartment and completely submerges it. The anode material occupies much of the space in the anode compartment on each side of the tunnel-like cathode compartment. In case it is desired to deposit layers of copper, the anode may be of "copper shot," or small balls, 29, resting between and against the walls of the cathode compartment 27 and copper plates 30, to which the positive lead from any suitable source of current electricity may be connected. To keep the electrolyte from teeming over the sides of the cell, drain pipes 31 are provided. These maintain the electrolyte during operation at a constant level which is above the top of the cathode chamber, and drain the overflow into the catch tank 11.

From compartment 31 in the elevated reservoir 12, electrolyte 25 sinks through the standpipe 16, gathering speed as it passes through the restriction 32 into the branches 33. Each branch 33 delivers to one of the nozzles 34, each of which is designed to have Venturi characteristics or such characteristics as to deliver the electrolyte entering it through the narrow entrance orifice 35 into the slot 23 and thence into the cathode tunnel at extremely high speed. As illustrated in Fig. 5, one nozzle 34 delivers into the slot at one side of the cathode ribbon 24, while the other nozzle delivers into the slot on the other side of said ribbon. The nozzles 34 are separated from each other by a narrow passage 36 of dimensions adapted to allow the cathode ribbon to move between them. Fig. 5 shows the nozzles view from above, the top plate having been partly broken away. They may be made of glass, vulcanite, acid-proof metal, glazed porcelain or other suitable material, and may be made integral or of parts cemented or fused together, according to convenience of manufacture. The communication between the high speed nozzle or nozzles and the cathode chamber is a closed one in order that the high pressure requisite to the required high speed of the electrolyte may be attained.

The electrolyte, delivered into the narrow cathode tunnel at exceedingly high speed on each side of the cathode ribbon, aids in keep-

ing the flexible ribbon centered in the tunnel, because the pressure is equal on both sides and quite adequate to straighten any slight bulges or bends in the metal ribbon. It travels at high speed and pressure. With the reservoir 12 elevated at from three to thirty feet, speeds of from ten to forty feet a second may be imparted to the electrolyte in the cathode compartment. All of the electrolyte enters the cathode compartment and the major portion of it passes through said compartment at high speed, emerging from the slot 23 in the rear end wall 21 of the cell. A minor portion of the electrolyte passes through the porous wall of the cathode compartment and enters the anode compartment, flowing through it much more slowly as a separate stream, said anode compartment in the illustrated embodiment being open to the atmosphere. The quantity of the electrolyte flowing through the anode compartment should be about ten per cent of that flowing in the cathode tunnel, and this percentage may be quite accurately attained by using a proper size of granules and suitable binder in the composition of the tunnel walls. None of the electrolyte in the anode compartment can rejoin the stream in the cathode compartment because of the high pressure existing in the latter.

As the pressure of the electrolyte drops only slightly in passing through the cathode compartment, once the full speed of the stream has been attained, it spurts from the slot 23 in the rear end wall 21 of the cell with great velocity. In order to dissipate the kinetic energy in the jetting stream of electrolyte, a baffling compartment 37 is provided at the rear end of cell 10. The rear wall 39 of this baffling compartment has a slot 38 which is in alignment substantially with the slots 23 in the end walls of the cell, through which the cathode strip travels. A removable plate 40 covers the upper side of compartment 37, and the rear wall 39 is cut away as at 41 so as to form an outlet or weir for the electrolyte that does not escape through the slot 38 around the cathode, but wells upward in the chamber. Another baffling compartment 42 having an opening at 43 in its bottom and having a rear wall 44, provided with a slot 45 for the passage of the now compound strip 24<sup>a</sup>, prevents the spattering about of the electrolyte issuing from the slot 38, which encounters the mass falling over the upper edge of wall 39 at the cut away part 41 and thereafter the rear wall 44 of the rear-most baffling chamber. The electrolyte issuing from the cathode compartment now drops through the lower opening 43 into the catch tank 11, to join with that flowing from the anode compartment through the overflow pipes 31.

Catch tank 11 preferably has a floor 46

that inclines downward toward a sump 45 at the forward end, whence the electrolyte is removed through the intake pipe 14 of the acid-proof pump 13, which forces it through the pipe 15 into the elevated reservoir 12.

5 The elevated reservoir 12 is shown as divided by a partition 47, which does not reach to the top of the reservoir, into compartments 48 and 31. Below the upper edge 10 of partition 47 there is shown a filter plate or layer 49, which may be composed of silica sand, granular carborundum or other suitable material. The electrolyte filters through said filter plate into the compartment 15 31, whence it falls by gravity into the standpipe 16. Thus the electrolyte may be purified of sediment by settling in the compartment 48 and by filtration in compartment 31.

20 The cathode 24, as before stated, may be of indefinite length. Commercial rolled strips of copper suitable for this use, five one-thousandths of an inch in thickness, are obtainable as long as 400 feet. Such a strip 25 in coil form may be mounted on spool 17, which may rotate with any desired frictional resistance on its stand 50. One end of said cathode strip may be threaded through the cell and attached to the reel 18. The reel 18, 30 to secure best results, should be evenly rotated at a speed predetermined according to the thickness of deposit required and the current density utilized. I have shown, somewhat conventionally, a power drive comprising a motor 51, the speed of which 35 may be accurately controlled driving, through a reducing gear if desired, a worm 52 in mesh with a worm wheel 53 on vertical shaft 54 with which the reel 18 rotates.

40 The cathode strip may be coated with any of the coatings usually applied to cathode surfaces. Sodium sulphide has been found satisfactory for the purpose.

45 After the entire length of cathode ribbon has received a deposit on both sides and been wound up on the reel 18, the coil of compound or three-layered metallic strip may be removed, treated as desired, and the layers stripped from the cathode ribbon as independent strips or sheets of the required metal.

The apparatus operates in a manner, which will now be clear, to carry out the process heretofore described.

55 It will be perceived that the electrolyte flows through the cell in two streams of differential pressure, the high pressure stream flowing in contact with the cathode and the low pressure stream flowing in contact with 60 the anode or anode material; that the cathode is inclosed and completely separated from the anode material by a partition freely permeable to the electric current but more difficultly permeable to the electrolyte; 65 that almost any pressure desired, subject to

limitations imposed by the strength of materials used, may be obtained in the cathode compartment and therefore very high speeds of replacement of electrolyte in contact with the cathode attained; no electrolyte in the 70 anode compartment can unite with the stream in the cathode compartment owing to the difference of pressure in the two streams. Thus extremely high density currents, far above 300 amperes per square foot, can be 75 utilized for the rapid production of electrolytic deposits.

A system composed of a plurality or battery of units of the kind described effects great economies in electro-deposition of 80 metals as compared with the usual practice using relatively low current densities. Very much less space is required for the same output, less electrolyte need be used, a much smaller reserve supply of anode metal need 85 be kept on hand, and less labor is required.

Each cell is only a small fraction of the size of that which would have to be employed where the usual low current densities are utilized. The amount of electrolyte in 90 use can be reduced. In proportion as the current density is increased. The amount of "dead" metal in the form of anode material necessary to be kept in reserve can be very much reduced. The amount of labor 95 and supervision necessary for a given output per day is less. The great expense of maintaining highly polished cylindrical cathodes, of great size (usual in the production of long strips electrolytically) is entirely eliminated, since in this process a 100 standard rolling mill product may be used, which, if it becomes damaged, can be worked up into standard manufactured products.

Although for purposes of exemplification 105 I have illustrated and described a specific apparatus for practicing the process of this invention, it will be understood that the apparatus may be modified in details, changed in position or improved, without departing 110 from the spirit of my invention, which is not intended to be limited to details described but only by the appended claims.

What I claim and desire to secure by Letters Patent of the United States is: 115

1. The process of depositing metal electrolytically upon a cathode surface, using extremely high cathode current densities, which consists in completely separating the anode and cathode in the cell by a semi-permeable, non-conducting partition of low electrical resistance when saturated with electrolyte, thereby forming two compartments affording no passage for electrolyte from one to the other except through said 120 partition, and forcing electrolyte through the cell in two streams under differential pressures, the higher pressure being in the cathode compartment.

2. A process of depositing metal electrolyt- 125

ically upon a cathode surface, using extremely high cathode current densities, which consists in completing separating the anode and cathode in the cell by inclosing the cathode in a tunnel-like compartment having a wall of porous, non-conducting material, semi-permeable to the electrolyte and of low electrical resistance when saturated with electrolyte, thereby forming two compartments affording no passage for electrolyte from one to the other except through said wall and circulating the electrolyte continuously through the cell in two streams under differential pressures, the higher pressure being in the cathode compartment.

3. The process of depositing metal electrolytically upon a cathode surface, using extremely high cathode current densities, which consists in completely separating the anode and cathode in the cell by porous, non-conducting partition, semi-permeable to the electrolyte and of low electrical resistance when saturated with electrolyte, thereby forming two compartments, affording no passage for electrolyte from one to the other except through said partition, forcing the electrolyte through the cell in two distinct streams, the major portion being forced at high pressure and high speed through the cathode compartment, which is closed except where the electrolyte enters and leaves it, and the lesser portion being forced through the partition and through the anode compartment, which is open and at atmospheric pressure.

4. The process of depositing metal electrolytically upon a cathode surface, using extremely high cathode current densities, which consists in enclosing the cathode in a tunnel-like compartment, thereby completely separating the cathode from the anode in the cell, said compartment having a wall of porous, non-conducting material, semi-permeable to the electrolyte and of low electrical resistance when saturated with the electrolyte thereby forming two compartments affording no passage for electrolyte from one to the other except through said wall, and forcing the electrolyte through the cell in two distinct streams, the major portion being forced at high pressure and high speed through the cathode-enclosing compartment, and the lesser portion being forced through the wall of said cathode compartment, and through the anode compartment, which is under lower pressure than the cathode compartment.

5. The process of depositing metal electrolytically upon a cathode surface, using extremely high cathode current densities, which consists in completely separating the anode and cathode in the cell by a porous, non-conducting partition, semi-permeable to the electrolyte and of low electrical resistance when saturated with electrolyte, forcing

the electrolyte through the cell in two distinct streams, the major portion being forced at high pressure and at a speed of not less than ten feet per second through the cathode compartment, which is closed except where the electrolyte enters and leaves it, and the lesser portion being forced through the anode compartment, which is under lower pressure than the cathode compartment.

6. The process of depositing metal electrolytically upon a cathode surface, which consists in using cathode current densities in excess of 300 amperes per square foot, completely separating the anode and cathode in the cell by a porous, non-conducting partition, semi-permeable to the electrolyte and of low electrical resistance when saturated with electrolyte, forcing the electrolyte through the cell in two distinct streams, the major portion being forced at high pressure and high speed through the cathode compartment, which is closed except where the electrolyte enters and leaves it, and the lesser portion being forced through the anode compartment, which is under lower pressure than the cathode compartment.

7. The process of depositing metal electrolytically upon a cathode surface, using extremely high cathode current densities which consists in completely separating the anode and cathode in a cell by enclosing an elongated cathode of ribbon form in a tunnel-like compartment, having a porous, non-conducting wall, semi-permeable to the electrolyte and of low electrical resistance when saturated with electrolyte, said tunnel conforming in cross section to the form of the cathode and being but slightly larger than said cathode, and forcing the major portion of the electrolyte at high pressure and high speed into the said tunnel on both sides of the ribbon cathode, in order to center the same within the tunnel.

8. The process of depositing metal electrolytically upon a cathode surface, using extremely high cathode current densities, which consists in completely separating the anode and cathode in the cell by enclosing an elongated, flexible cathode of ribbon form in a tunnel-like compartment of porous, non-conducting material, semi-permeable to the electrolyte and of low electrical resistance when saturated with electrolyte, said tunnel-like compartment conforming in cross section to the form of the cathode and being slightly larger in cross section than the cathode, and forcing the electrolyte through the cell in two distinct streams, the major portion being forced at high pressure and high speed through the cathode compartment on both sides of the cathode, thereby centering it in the compartment, and the lesser portion being forced through the anode compartment, which is under lower pressure than the cathode compartment.

9. The process of depositing metal electrolytically upon a cathode surface, which consists in completely separating the cathode from an anode by a semi-permeable non-conducting partition of low electrical resistance when saturated with electrolyte thereby forming two compartments affording no passage for the electrolyte from one to the other except through said partition and applying electrolyte moving at high speed to the cathode surface while maintaining a pressure on the cathode side of the partition higher than that on the anode side.

10. In an electrolytic apparatus, a cell comprising an anode and a cathode compartment completely separated by a porous partition of non-conducting material semi-permeable to the electrolyte and of low electrical resistance when saturated with electrolyte, means for maintaining a difference of pressure between said anode and cathode compartments in favor of the latter, and means for more rapidly renewing the electrolyte in contact with the cathode than the electrolyte in contact with the anode or anodes is renewed.

11. In an electrolytic apparatus, a cell, comprising an anode compartment and a cathode compartment consisting of a tunnel passing through said anode compartment from end to end, said cathode compartment having a porous wall of non-conducting material, semi-permeable to the electrolyte and of low electrical resistance when saturated with electrolyte.

12. In an electrolytic apparatus, a cell, comprising an anode compartment and a cathode compartment consisting of a tunnel passing through said anode compartment from end to end, said cathode compartment having a porous wall of non-conducting material, semi-permeable to the electrolyte and of low electrical resistance when saturated with electrolyte, and a cathode within said compartment, said compartment being of a cross section corresponding to the cross section of the cathode, and but slightly larger.

13. In an electrolytic apparatus, a cell, comprising an anode compartment and a cathode compartment consisting of a tunnel passing completely through said anode compartment and open at each end at the exterior of the cell, said cathode compartment having a porous wall of non-conducting material, semi-permeable to the electrolyte and of low electrical resistance when saturated with electrolyte, the passage through said tunnel being of an oblong form in cross section, and a ribbon form cathode inclosed within said tunnel and nearly filling it, there being spaced wear-resisting guides, of material inert to the electrolyte, for guiding and centering the ribbon cathode.

14. In an electrolytic apparatus, a cell, comprising an anode compartment and a

cathode compartment, completely separated from each other by a porous wall of non-conducting material, semi-permeable to the electrolyte and of low electrical resistance when saturated with electrolyte, said cathode compartment being completely closed except that it is provided with an inlet and outlet for admitting and discharging electrolyte, and means comprising a nozzle in closed communication with the cathode compartment for forcing electrolyte under pressure into the inlet opening and through said cathode compartment.

15. In an electrolytic apparatus, a cell, comprising an anode compartment and a cathode compartment consisting of a tunnel passing completely through said anode compartment and open at each end at the exterior of the cell, said cathode compartment having a porous wall of non-conducting material, semi-permeable to the electrolyte and of low electrical resistance when saturated with electrolyte, the passage through said tunnel being of an oblong form in cross section, and a ribbon form cathode inclosed within said tunnel and early filling it, a pair of nozzles, one on each side of the ribbon cathode, and means for forcing the electrolyte through said nozzles, under pressure, into said tunnel.

16. In an electrolytic apparatus, a cell, comprising an anode and a cathode compartment, completely separated from each other by a porous wall of non-conducting material, semi-permeable to the electrolyte and of low electrical resistance when saturated with electrolyte, said cathode compartment being completely closed except that it is provided with an inlet and outlet for admitting and discharging electrolyte, and a slotted baffling chamber in communication with the outlet, adapted to dissipate the kinetic energy of the outflowing electrolyte and prevent spalshing.

17. In an electrolytic apparatus, a cell, comprising an anode and a cathode compartment, completely separated from each other by a porous wall of non-conducting material, semi-permeable to the electrolyte and of low electrical resistance when saturated with electrolyte, said cathode compartment being completely closed except that it is provided with an inlet and outlet for admitting and discharging the electrolyte, and a slotted baffling chamber in communication with the outlet, adapted to dissipate the kinetic energy of the outflowing electrolyte and prevent splashing, said chamber having a weir-like orifice at its upper portion for permitting outflow of the electrolyte.

18. In an electrolytic apparatus, a cell, comprising an anode and a cathode compartment, completely separated from each other by a porous wall of non-conducting

material, semi-permeable to the electrolyte and of low electrical resistance when saturated with electrolyte, said cathode compartment being completely closed except that it is provided with an inlet and outlet for admitting and discharging the electrolyte, a slotted baffling chamber in communication with the outlet, adapted to dissipate the kinetic energy of the outflowing electrolyte and prevent splashing, said chamber having a weir-like orifice at its upper portion for permitting outflow of the electrolyte, and a slotted baffle plate in rear of the baffling chamber.

15 19. In an electrolytic apparatus, a cell, comprising an anode and a cathode compartment, completely separated from each other by a porous wall of non-conducting material, semi-permeable to the electrolyte and of low 20 electrical resistance when saturated with electrolyte, said cathode compartment being completely closed except that it is provided with an inlet and outlet for admitting and discharging the electrolyte, a catch-pan 25 underneath the cell adapted to receive electrolyte discharged therefrom, a tank elevated above the cell, a pump for delivering electrolyte from the pan to the tank, and an outlet from the tank in closed communication with the inlet of the cathode chamber.

30 In testimony whereof, I hereto affix my signature.

HERBERT C. HARRISON.

35

40

45

50

55

60

65